

## UNITED STATES PATENT OFFICE

1,965,093

## ALLOY

Julius Aderer, New York, N. Y.

No Drawing. Application March 18, 1933,  
Serial No. 661,637

2 Claims. (Cl. 75—1)

The object of the invention is to provide a new alloy composed essentially of the precious metals, palladium and gold, and more particularly for the purpose of providing dental auxiliary elements for oral installation constituted of an alloy suitable for dental purposes shaped in the form of wires, bands, crowns, plates, etc. for appropriate application with reference to the dental condition in connection with which the auxiliary elements are to be used.

Heretofore, in the manufacture of such dental auxiliary elements it has been customary to use alloys in which the percentage of gold predominates over the percentage of all other metals, the gold being ordinarily alloyed with relatively large quantities of platinum of the order of 10% to 22%. Such alloys, while capable of use for their intended purposes, are necessarily expensive.

20 I have discovered that if the platinum is entirely omitted or permitted to be present only in small percentages of the order of less than 10%, and if a smaller amount of gold is alloyed with a larger proportion of palladium, the alloy also 25 containing copper, some silver, and zinc, a superior alloy for dental purposes can be produced at a cost which is approximately half that of the gold-platinum alloys.

In perfecting the composition of the new alloy 30 it was necessary to bear in mind that the alloy must have a high fusing point which is essential for soldering. Although platinum has a higher fusion point than palladium, the fusion point of an alloy of palladium and gold is higher than 35 that of an alloy of platinum and gold. As an increase in the percentage of palladium in the alloy raises its fusion point, and the palladium also possesses or imparts a desirable color, I use an excess of palladium over the amount of gold.

40 Copper forms a part of the alloy to impart to it the quality of hardness, while zinc, imparts the necessary elasticity and toughness. The alloy possesses the requisite high fusing point, the quality of not losing color in the mouth, and 45 sufficient strength.

This alloy can be rolled from bars say fifteen 50 inches long and one-fourth inch square to wires approximately one-sixteenth inch square. This can be accomplished without annealing and the alloy does not show any fatigue during the rolling process. Any other comparable metal alloy 55 will break under similar treatment. The property possessed by the new alloy is therefore valuable in saving labor. The new alloy can also be drawn through diamond draw plates to approxi-

mately twelve-thousandths of an inch, which is as fine as is required for dental uses. The wires or other forms may be annealed but in that case temperatures above 1200° F. and preferably of the order of 1800° F. or upwards should be employed. This treatment softens the wire and takes the springiness or elasticity out of it. After such annealing the wire can be readily shaped and the dental attachments soldered thereto. Thereupon the dentist heats the product to about 60 65 1000° F. and allows it to cool slowly. This treatment tempers the finished product. The wires made of the new alloy possess a high degree of elasticity and will not snap unless very sharply bent.

70 The new alloy is easily produced, the zinc, copper, and silver being placed in a furnace or crucible, usually in the form of small pellets, the zinc first, copper on top, and then silver. The gold and palladium are first thoroughly mixed in a 75 separate crucible and the mixture is rolled out and then put into the crucible containing the zinc, copper, and silver.

A formula which I have found extremely satisfactory is: gold approximately 33½ parts, silver 80 approximately 5 parts, palladium approximately 39 parts, copper approximately 22 parts, and zinc approximately 4 parts. The amount of gold may very between the limits of 30 to 40 parts, the palladium between about 35 to 50 parts, the 85 copper between about 18 to 30 parts, the silver about 5 to 8 parts, and the zinc between about 2 to 6 parts. The amount of silver may be increased, for instance, as set forth in my Patent No. 1,924,097, dated August 29, 1933, to approximately between 10 to 23 parts. The silver is present in the new alloy in order to obtain a more homogeneous alloy, but with careful manipulation it is possible to obtain an alloy of equal value without using silver at all.

15 The addition of some platinum not in excess of 10% will not defeat the advantage of the new alloy, though it is preferred to have no platinum present. In other words I desire it to be understood that if some platinum, not in excess of 100 10% is added, the presence of such material would not alter the essential character of my new alloy.

The melting point of my new alloy is about 105 2085° F. The Brinell hardness in the softened state is about 202; after tempering at 860° F., and cooling it slowly in thirty minutes, the alloy showed a Brinell hardness of about 426. The tensile strength of this wire, when tempered, is as high as 191,000 pounds per square inch. When 110

it is annealed or softened, the tensile strength is only between 88,000 and 103,600, showing an elongation between 25 and 28 in 2 inches, whereas in the hardened state the elongation is only 5 from 2 to 5.

This new alloy combines with a high fusing point, which is very desirable, an elastic quality of a high degree.

I claim:

10 1. An alloy constituted of approximately 30 to 40 parts gold, approximately 35 to 50 parts pall-

dium, approximately 18 to 30 parts copper, and approximately 2 to 6 parts zinc.

2. A dental auxiliary element for oral installation in the form of a shaped member conformable to a dental condition, said element being constituted of an alloy composed of approximately 30 to 40 parts gold, approximately 35 to 50 parts palladium, approximately 18 to 30 parts copper and approximately 2 to 6 parts zinc.

80

85

JULIUS ADERER.

15

90

20

95

25

100

30

105

35

110

40

115

45

120

50

125

55

130

60

135

65

140

70

145

75

150